

## UNITED STATES PATENT OFFICE

2,075,757

## METAL TREATMENT

Victor Conquest, Chicago, Ill., assignor to Armour and Company, Chicago, Ill., a corporation of Illinois

No Drawing. Application June 29, 1936, Serial No. 88,066

20 Claims. (Cl. 91—68)

This invention relates to the treatment of metal surfaces to provide them with a corrosion-resisting film and it comprises, as new products, metal articles carrying a corrosion-resistant film composed of a ketone having the general formula



10 wherein R is a closed ring radical and R' is an aryl radical containing at least six carbon atoms; it further comprises processes wherein metal surfaces subject to atmospheric corrosion are coated with such ketones.

15 Various methods of providing metal surfaces such as steel with corrosion-resisting coatings have been proposed in the prior art. For example, steel has been treated with many different chemical reagents to so modify the steel surface that an anti-rusting surface is presented 20 to the forces of atmospheric corrosion. Such metal treatment results in the deposition on the surface of an extremely thin film which is not attacked by atmospheric moisture, oxygen, and similar substances ordinarily tending to rust the 25 steel. All of these so-called metal treatments are essentially surface reactions. They are not to be confused with painting or otherwise applying 30 protecting coatings which do not actually modify the surface of the metal itself. Paints and like coating compounds merely form a coating on the surface. Should the paint chip off, the exposed metal surface rusts or corrodes readily.

These metal treating processes are of great 35 utility in the pre-treatment of metal surfaces prior to the application of ornamental paint films. For example, it is customary to "rust-proof" steel automobile bodies before the application of lacquers thereto. This is to protect the metal surface in the event some of the lacquer 40 film is chipped or scratched off.

I have now discovered that so-called "mixed 45 ketones", that is, ketones wherein one of the radicals attached to the carbonyl group is a closed ring radical such as phenyl, and the other radical is an alkyl radical containing at least six 50 carbon atoms, will form adsorbed molecular films on metal surfaces normally corroding or rusting in the atmosphere, that such films are substantially permanent, and that such films protect the metal surface against corrosion. These films are not, however, to be confused with 55 coatings such as lacquers. Apparently metal surfaces treated with the ketones of my invention actually unite with the ketone in some way. This

can be demonstrated quite readily. When steel articles, such as automobile fenders, are immersed in, or sprayed with a liquid mixture of ketones of the class embraced within my invention, and the surface then drained to remove excess ketone so that the surface is apparently free of any extraneous material, the metal is highly anti-corrosive. In fact when the treated metal surfaces are actually subjected to the action of good solvents for the ketone films thereon, the 10 film cannot be removed. This indicates to me that the metal surface has adsorbed a thin film, probably of molecular dimensions. Adsorption phenomena of this type are in the realm of 15 surface chemistry and cannot, of course, be predicted. That the metal surface will adsorb molecular films of these ketones is surprising although the adsorption of gas, liquids and solids by surfaces is, of course, a recognized physical-chemical phenomenon.

20 The ketones which I use to protect the metal against corrosion are all highly stable substances chemically. They are insoluble in water and are not oxidized by air, moisture, light, or carbon dioxide and similar acidic compounds normally 25 present in the atmosphere. Their inertness toward atmospheric influences makes them especially useful in the practice of my invention. Moreover, they are relatively inexpensive since 30 they can be prepared from the cheap fatty acids available in large quantities.

When practising my invention all that is necessary is to cause the metal surface to contact with the ketone in any suitable manner. As will be pointed out in detail presently, all of the ketones used in my invention are either liquids or wax-like solids. When using normally liquid ketones for the treatment of the metal surface, I simply immerse the metal article in a bath of the ketone or mixtures thereof, and wipe off, or drain off, 40 any excess liquid. Surface adsorption is almost instantaneous. Phenyl hexyl ketone is liquid and is a satisfactory material to use. One of the best ketonic compounds is that prepared from commercial xylene and higher fatty acid chlorides derived from lard fatty acids in ways well known. This ketonic material is a mixture of ketones in which the aryl radical is a mixture of meta and para xylol. In other words, the ketonic mixture is a mixture of isomeric xylol-alkyl ketones having at least eight or ten carbon atoms in the alkyl radical. As stated, this mixture is liquid at temperatures as low as 0° C. and the metal article can be immersed therein, or the metal surface can be sprayed with the ketonic material.

5

15

20

25

30

35

40

45

50

55

Other ketones in the list which I shall presently give are solids. When using such ketones they can be melted and the metal article immersed in the molten liquid. All of my ketones are soluble 5 in hydrocarbon solvents and in some cases it is convenient to dissolve a normally solid ketone in such a solvent and spray the metal article with the solution.

After forming an adsorbed surface film on the 10 metal article the coated surface can then be painted, lacquered or otherwise ornamented with coating compounds in ways well known. All of the usual coating compounds adhere strongly to the pre-treated surface.

15 I shall now list many ketones which can be used in the practice of my invention. For economic reasons many of these ketones would not be used since they are somewhat expensive in comparison with ketones like the above-described 20 mixtures of xylol-alkyl ketones, the phenyl-heptadecyl ketones, and others produced in part from benzene and naphthalene. But in order to indicate the breadth of my invention, I am listing many different types of ketones falling within my 25 generic disclosure. As stated, in most instances I find it more economical to use the cheap ketones, or various mixtures thereof, such as phenyl heptadecyl ketone, mixtures thereof with xylol heptadecyl ketone, etc. Proportions in such mixtures 30 are not at all critical; whether mixtures are to be used will be governed largely by the cost of the ketones.

A representative list of ketones I can use is as follows:

- 35 Phenyl heptadecyl ketone
- p-Tolyl heptadecyl ketone
- m-Xylol heptadecyl ketone
- p-Xylol heptadecyl ketone
- m-Xylol pentadecyl ketone
- p-Tolyl pentadecyl ketone
- p-Methoxyphenyl pentadecyl ketone
- p-Ethoxyphenyl pentadecyl ketone
- Phenyl undecyl ketone
- p-Chlorophenyl undecyl ketone
- p-Methoxyphenyl heptadecyl ketone
- p-Methoxyphenyl undecyl ketone
- p-Phenoxyphenyl heptadecyl ketone
- p-Phenoxyphenyl tridecyl ketone
- p-Phenoxyphenyl undecyl ketone
- p-Nitro phenoxyphenyl heptadecyl ketone
- p-Methyl phenoxyphenyl heptadecyl ketone
- Alkyl phenones from lard fatty acids.
- Alpha naphthyl heptadecyl ketone
- Alpha naphthyl pentadecyl ketone
- Anthracyl heptadecyl ketone (mixtures)
- Biphenyl heptadecyl ketone
- Biphenyl tridecyl ketone
- Biphenyl undecyl ketone
- 60 p-Methyl biphenyl heptadecyl ketone
- p-Chlorobiphenyl heptadecyl ketone
- Furyl heptadecyl ketone
- Furyl undecyl ketone
- Methyl furyl heptadecyl ketone
- 65 Dibenzofuryl heptadecyl ketone
- Dibenzofuryl undecyl ketone.

Consequently, in the appended claims I define my ketonic materials broadly as those in which 70 one of the radicals attached to carbonyl is a closed ring radical and the other is an alkyl radical having at least six carbon atoms.

Likewise, in the appended claims I wish to define the metal treated broadly. Apparently all 75 metals will adsorb molecular layers of my ketonic

materials and such adsorbed films prevent corrosion of the metal surface. My experiments demonstrate that this action takes place on steel, iron, copper, aluminum, nickel, chromium, and other common metals. Many of these metals, or 5 their alloys do not however corrode or rust as readily as iron or steel. Copper and aluminum will, of course form oxide layers unless otherwise protected and my invention can be used to keep copper from discoloring as a result of atmospheric influences. My invention is especially useful in the treatment of steel and iron surfaces, and it can even be used to prevent silver from tarnishing. Silver articles tarnish readily due to contact with hydrogen sulphide in the 10 atmosphere. An adsorbed layer of ketonic material on the silver prevents this. Since the ketonic films are of molecular dimensions they cannot, of course, be detected by visual inspection 15 and the treated silver does not have a greasy or waxy feel.

It will be apparent that many other metal 20 surfaces are benefited by the processes of the present invention. Ornamental aluminum on the exterior of buildings can be kept shiny if pre-treated with my ketones prior to exposure 25 to the atmosphere. Aluminum foil, and other metal foils used for heat insulation can be maintained shiny so that a maximum amount of heat is radiated.

Having thus described my invention what I 30 claim is:

1. A metal article having a surface provided 35 with a corrosion-resisting film of a ketonic material composed of at least one ketone having the formula



40 wherein R is a closed ring compound and R' is an alkyl radical having at least six carbon atoms.

2. The article as in claim 1 wherein R is an 45 aryl group.

3. The article as in claim 1 wherein R is a phenyl radical.

4. The article as in claim 1 wherein R is a xylol radical.

5. The article as in claim 1 wherein the 50 ketonic material is a mixture of isomeric xylol-alkyl ketones in which the alkyl group contains at least eight carbon atoms.

6. A steel article having a surface provided 55 with a corrosion-resisting film of a ketonic material composed of at least one ketone having the formula



60 wherein R is a closed ring compound and R' is an alkyl radical having at least six carbon atoms.

7. The article as in claim 6 wherein R is an aryl group.

8. The article as in claim 6 wherein R is a phenyl radical.

9. The article as in claim 6 wherein R is a xylol radical.

10. The article as in claim 6 wherein the 70 ketonic material is a mixture of isomeric xylol-alkyl ketones in which the alkyl group contains at least eight carbon atoms.

11. The process of protecting the surface of 75 metals against corrosion which includes treat-

ing the surface with a ketonic material composed of at least one ketone having the formula



5 wherein R is a closed ring compound and R' is an alkyl radical having at least six carbon atoms.

12. The process as in claim 11 wherein R is an aryl group.

10 13. The process as in claim 11 wherein R is a phenyl radical.

14. The process as in claim 11 wherein R is a xylyl radical.

15 15. The process as in claim 11 wherein the ketone is a mixture of isomeric xylyl-alkyl ketones in which the alkyl group contains at least eight carbon atoms.

16. The process of protecting the surface of steel articles against corrosion which includes

treating the surface with a ketonic material composed of at least one ketone having the formula



5

wherein R is a closed ring compound and R' is an alkyl radical having at least six carbon atoms.

17. The process as in claim 16 wherein R is a phenyl radical.

18. The process as in claim 16 wherein R is a phenyl radical.

19. The process as in claim 16 wherein R is a xylyl radical.

20. The process as in claim 16 wherein the ketone is a mixture of isomeric xylyl-alkyl ketones 15 in which the alkyl group contains at least eight carbon atoms.

VICTOR CONQUEST.